

## UNITED STATES PATENT OFFICE

2,516,616

## LUBRICATING OIL DETERGENT

James O. Clayton, Berkeley, and Dorr H. Etzler, Albany, Calif., assignors to California Research Corporation, San Francisco, Calif., a corporation of Delaware

No Drawing. Application December 30, 1947,  
Serial No. 794,810

15 Claims. (Cl. 252—33.6)

1

This invention relates to reducing the formation of gum deposits resulting from the deterioration of lubricating oils by incorporating therein certain salts of selenium-containing acids.

Ordinarily, lubricating oils deteriorate and, in general, form gums when they are exposed to oxygen at elevated temperatures. For example, crankcase oils, transmission oils, and the like have a tendency to break down during the operation of engines, resulting in the formation of gums. The gums which are formed collect in the oil rings and the oil lines to cause the sticking of the piston rings and to inhibit the free flow of the lubricating oil. Thus, the parts of the motors and gears requiring lubrication suffer from the lack of proper lubrication. In order to reduce the formation of gum deposits, it is essential to incorporate certain agents to serve as detergents. The presence of detergents reduces the formation of gum deposits and permits the parts of an engine, for example, to receive the proper lubrication, eliminating unnecessary wear of parts due to improper lubrication.

Many of the internal combustion engines of today operate at higher temperatures and higher compressions than heretofore with a resulting greater stress upon the lubricating oils and the more rapid deterioration of these oils. Thus, modern internal combustion engines, especially those of the Diesel type, become fouled and develop piston ring sticking more quickly than did the older type engines when lubricated by the same oil. To complicate matters even still further, certain of the bearings of the engines of today bear greater loads and are of the hard alloy type, such as cadmium-silver and copper-lead bearings. The greater loads on bearings demand better lubricant performance. Although the hard alloy bearings mentioned above are preferred to the old babbitt bearings from the mechanical standpoint, the hard alloys are more readily corroded by certain mineral oils, by used oils in which acidic products of oxidation have accumulated and by the action (believed to be an indirect, catalytic action rather than a direct corrosive action) of certain additives, such as calcium stearate and calcium naphthenate which are sometimes added to oils to inhibit piston ring sticking and the like.

It is an object of this invention to provide an addition agent for hydrocarbon lubricating oils which will reduce the deposits of gums from the lubricating oils.

It is another object of this invention to provide an agent which is a detergent for the gums formed in lubricating oils.

2

It is a further object of this invention to provide useful compounds of selenium capable of improving hydrocarbon oils.

These and other objects will be apparent from the following description and claims.

In accordance with the invention, there is incorporated in a lubricating oil a small amount of a polyvalent metal salt of seleninic acid of the following formula:



wherein R may be an aliphatic radical, an alkaryl radical or an aralkyl radical. The R radical may contain, as substituents, polar groups such as chlorine, bromine, hydroxyl, ether, keto, mercapto, etc.

The base substance in which the polyvalent metal salt of the seleninic acid is incorporated will normally be petroleum lubricating oils and synthetic oils of lubricating viscosity. These oils may range in viscosity from spindle oils to cylinder stocks.

The polyvalent metal cations of the salts of this invention are the metals of Groups II, III, IV and VI of the periodic table, specifically, calcium, strontium, barium, cadmium, zinc, aluminum, chromium, lead and tin. It is preferred to use calcium, barium and zinc metal salts, since these are more effective detergents than the salts of the other metals listed hereinabove.

In the above formula, the R may be an alkyl radical, an aralkyl radical or an alkaryl radical. These radicals may be straight-chained, branch-chained, saturated or unsaturated, containing from 10 to 40 carbon atoms. It is preferred to use straight-chained, saturated aliphatic radicals having from 12 to 24 carbon atoms. The R group may be exemplified by the following radicals: decyl, dodecyl, tetradecyl, cetyl, octadecyl, tetracosyl, dotriacosyl, isoamyl phenyl, tributyl phenyl, cetyl phenyl, amyl naphthyl, etc.

Ordinarily, to effect detergency in a lubricating oil, the amount of a salt of a seleninic acid which is included in the oil composition will depend on the oxidation load of the composition. That is, an oil composition which is used under conditions resulting in large amounts of oxidation products being formed in the oil composition will require larger amounts of salts of seleninic acids to disperse the gums (oxidation products) formed than an oil composition which is used under such conditions that only small amounts of gums are formed.

The salts of the seleninic acids of this invention may be used in amounts as low as 0.1% or

less or as high as 2% or more. Preferably, 0.2% to 1% of a salt of a seleninic acid will be used in the practice of this invention. All percentages are by weight based on finished composition.

Concentrates or stock solutions containing 2% to 50% or more of a metal salt of a seleninic acid dispersed in an organic liquid (e. g., mineral lubricating oil) may be prepared for later blending with the substance to be stabilized to produce a finished product.

The following examples will illustrate the practice and the advantages of this invention:

*Example I.—Preparation of dodecane-1-seleninic acid*

64 milliliters of concentrated nitric acid ( $d=1.4$ ) was slowly added with stirring to 24.8 grams of pure didodecyl diselenide.<sup>1</sup> The temperature was maintained at approximately 50° C. for 10 minutes. Water was then added to the mixture to precipitate out the n-dodecyl seleninic acid. The product which was obtained had the following analysis:

| Theoretical for Dodecane-1-Seleninic Acid | Found   |
|-------------------------------------------|---------|
| Percent Se, 28.3                          | 28.1    |
| Equivalent Weight, 281.3                  | 281     |
| Melting Point                             | 80.5-81 |

*Example II.—Preparation of calcium dodecane-1-seleninate*

A solution of 20 grams of dodecane-1-seleninic acid in 95% alcohol was neutralized with 51% aqueous potassium hydroxide at room temperature to form the potassium salt. The calcium salt was precipitated by adding an excess of a 20% calcium chloride solution to the solution of potassium dodecane-1-seleninate.

*Example III.—Preparation of hexadecane-1-seleninic acid*

Twenty grams of crude n-hexadecyl selenocyanate was stirred with excess concentrated nitric acid ( $d=1.4$ ) for two hours at room temperature. This mixture was then kept standing at room temperature for 15 hours, then heated to 65° C. for three hours. When this mix was cooled to room temperature, the reaction product solidified and was separated from the aqueous layer by filtration. The crude hexadecane-1-seleninic acid was purified by crystallization from ethyl ether. The analysis of the resulting hexadecane-1-seleninic acid was as follows:

|                   | Calculated for<br>$C_{16}H_{34}SeO_2H$ | Found |
|-------------------|----------------------------------------|-------|
| Equivalent Weight | 337.5                                  | 338   |

*Example IV.—Preparation of calcium hexadecane-1-seleninate*

A solution of 44 grams of hexadecane-1-seleninic acid in 95% alcohol was neutralized with 51% aqueous potassium hydroxide at room temperature to form potassium hexadecane-1-selen-

<sup>1</sup> The didodecyl diselenide was prepared as follows: 10 grams of dodecyl seleno cyanate ( $C_{12}H_{24}SeCN$ ) was dissolved in 25 cc. of alcohol and the solution was cooled to 32° F. Two cc. of 50% aqueous NaOH were diluted with 10 cc. of alcohol and similarly cooled. On mixing the two solutions, a clear solution resulted which, however, began to deposit a solid in about 10 seconds and the solution then set to a solid. An additional 25 cc. of alcohol were stirred in and the mixture was allowed to stand at 40° F. for 2 hours. It was then poured into water and the oil that separated was extracted with ethyl ether. The ethyl ether extract was washed with water and dried over sodium sulfate and the ether removed by evaporation. The residue was crystallized from a mixture of ether and alcohol. The resulting product consisted of fine, pale yellow plates melting at about 21° C.

nate. An excess of a 20% calcium chloride solution was added to the solution of potassium hexadecane-1-seleninate to precipitate the calcium hexadecane-1-seleninate. The analysis of the calcium hexadecane-1-seleninate was as follows:

|            | Theoretical for<br>$(C_{16}H_{34}SeO_2)_2Ca$ | Found |
|------------|----------------------------------------------|-------|
| Percent Se | 22.2                                         | 19.8  |
| Percent Ca | 5.62                                         | 5.4   |

*Example V.—Preparation of octadecane-1-seleninic acid*

15 Sixty-five milliliters of concentrated nitric acid ( $d=1.4$ ) was slowly added with stirring to 34 grams of pure dioctadecyl diselenide at 50° C. The dioctadecyl diselenide was prepared according to the method in above Example I for didodecyl diselenide. The resulting mix was a paste, which was stirred for several hours at 50° C., then diluted with 300 milliliters of water to precipitate crude octadecane-1-seleninic acid, which was purified by crystallization from hot ethyl alcohol. The analysis of the octadecane-1-seleninic acid was as follows:

|                   | Calculated for<br>$C_{18}H_{36}SeO_2H$ | Found |
|-------------------|----------------------------------------|-------|
| Percent Se        | 21.6                                   | 21.7  |
| Equivalent Weight | 365.5                                  | 365   |
| Melting Point     | 93.5-94                                |       |

35 *Example VI.—Preparation of zinc octadecane-1-seleninate*

40 A solution of 25.4 grams of zinc acetate in 300 milliliters of 50% ethyl alcohol was added slowly with stirring to 96 grams of octadecane-1-seleninic acid in 300 milliliters of hot ethyl alcohol. Zinc octadecane-1-seleninate precipitated as a white finely divided substance which was washed in water and dried in vacuo over calcium chloride. The analysis of the zinc octadecane-1-seleninate was as follows:

|            | Theoretical for<br>$(C_{18}H_{37}SeO_2)_2Zn$ | Found |
|------------|----------------------------------------------|-------|
| Percent Se | 19.8                                         | 18.5  |
| Percent Zn | 8.2                                          | 7.7   |

55 The salts of this invention were compounded in a refined Western SAE 30 oil and tested in a Lauson gasoline engine. The test was carried out as follows: A single cylinder Lauson gasoline spark ignition engine, 2½ inch bore and 2½ inch stroke, loaded with a three-phase induction generator, was operated under extremely severe conditions designed to develop fully the tendency of the crankcase lubricant to deteriorate with gum formation and piston ring sticking. The engine was operated at 1200 revolutions per minute, the engine jacket temperature was maintained at 375° F., the crankcase oil was maintained at 300° F. and the engine was inspected after a 30 hour period of operation and after a 60 hour period of operation.

60 It appears that the polyvalent metal salts of seleninic acids (e. g., the zinc salts and the calcium salts) have greater detergent action than other detergent compounds (e. g., sulfonates) when used in lubricating oils.

65 Table I presents the test results obtained in a 70 Lauson engine test. The P. D. No. (Piston Dis-

coloration Number) as used in the Table I involves a careful inspection of the piston skirt to determine the degree of discoloration of the piston skirt. A completely black piston was assigned a P. D. No. of 800, and a completely clean piston was assigned a P. D. No. of 0. Piston discoloration numbers between 0 and 800 were given to pistons which ranged from totally clean to totally black.

Table I

| No. |                                               | Lauson Engine Test P. D. Number |          |
|-----|-----------------------------------------------|---------------------------------|----------|
|     |                                               | 30 Hours                        | 60 Hours |
| (1) | Western SAE 30 Base Oil                       | 615                             | -----    |
| (2) | Base Oil+0.3% Calcium Hexadecane-1-Seleninate | 425                             | -----    |
| (3) | Base Oil+0.6% Zinc Octadecane-1-Seleninate    | 50                              | 110      |

The polyvalent metal salt of seleninic acid compounding of the invention may be used as the only compounding, or it may be used in conjunction with other compounding agents, such as organic sulfides (e. g., dicetyl sulfide); sulfonates, such as calcium alkylbenzene sulfonate; phosphates (e. g., zinc cetylphenyl thiophosphate); phenates (e. g., calcium cetylphenate), etc.

In addition to the polyvalent metal salt of a seleninic acid, the finished oils of the invention may contain other agents, such as extreme pressure agents, blooming agents, pour point inhibitors, etc.

We claim:

1. A composition of matter consisting essentially of a major proportion of a mineral lubricating oil which is susceptible to deterioration when exposed to oxygen and, in an amount sufficient to improve the detergency of said lubricating oil a polyvalent metal salt of a seleninic acid.

2. The composition of claim 1, wherein said lubricating oil is a petroleum lubricating oil.

3. The composition of claim 1, wherein said polyvalent metal salt is a salt of a metal of the second group of the Periodic Table.

4. A composition of matter consisting essentially of a major proportion of a hydrocarbon oil which is susceptible to deterioration when exposed to oxygen and a small amount, sufficient to improve the detergency of said lubricating oil, of a polyvalent metal salt of a seleninic acid having a direct carbon to selenium linkage, said seleninic acid containing at least 10 carbon atoms.

5. The composition of claim 4, wherein said lubricating oil is a petroleum lubricating oil.

6. The composition of claim 4, wherein said polyvalent metal is zinc.

7. The composition of claim 4, wherein said polyvalent metal is calcium.

8. The composition of claim 4, wherein said polyvalent metal is barium.

9. The composition of claim 4, wherein said seleninic acid is hexadecane-1-seleninic acid.

10. The composition of claim 4, wherein said seleninic acid is octadecane-1-seleninic acid.

11. The composition of claim 4, wherein said seleninic acid is dodecane-1-seleninic acid.

12. A lubricant comprising a major portion of a mineral oil of lubricating viscosity and about 0.1% to 2% by weight based on the finished lubricant of a polyvalent metal salt of a seleninic acid of the formula



wherein the R is an alkyl radical containing from 10 to 40 carbon atoms.

13. A lubricant of claim 12, wherein said polyvalent metal salt of a seleninic acid is calcium hexadecane-1-seleninate.

14. A lubricant of claim 12, wherein said polyvalent metal salt of a seleninic acid is zinc octadecane-1-seleninate.

15. A lubricant comprising a major portion of a mineral oil of lubricating viscosity and about 0.1% to 2% by weight based on the finished lubricant of a polyvalent metal salt of a seleninic acid of the formula



35 wherein the R is an organic radical selected from the group consisting of alkyl and alkaryl radicals, said organic radical containing from 10 to 40 carbon atoms.

JAMES O. CLAYTON.  
DORR H. ETZLER.

#### REFERENCES CITED

The following references are of record in the file of this patent:

#### UNITED STATES PATENTS

Number Name Date  
2,350,783 Lincoln ----- June 6, 1944

#### FOREIGN PATENTS

Number Country Date  
2,787 Great Britain ----- of 1914

#### OTHER REFERENCES

Text Book of Inorganic Chemistry, vol. XI, part IV by Goddard; Chas. Griffin & Co., 1937, pp. 15 and 16 pertinent.